

# UNITED STATES PATENT OFFICE.

WILLIAM A. MCADAMS, OF BAY SHORE, NEW YORK.

## ALUMINUM ALLOY AND METHOD OF PRODUCING THE SAME.

1,095,653.

Specification of Letters Patent.

Patented May 5, 1914.

No Drawing.

Application filed October 2, 1913. Serial No. 792,983.

To all whom it may concern:

Be it known that I, WILLIAM A. MCADAMS, a citizen of the United States, and resident of Bay Shore, in the county of Suffolk and 5 State of New York, have invented a new and useful Improvement in Aluminum Alloys and Methods of Producing the Same, of which the following is a specification.

My invention consists in an aluminum alloy and in the method of producing the same, the said alloy comprising a novel combination of materials in novel proportions, producing a composition of matter especially well adapted for casting under pressure in 10 die-casting machines, said composition being very strong and resonant and having a permanent superior luster.

The alloy is composed of aluminum, zinc, copper and antimony combined in substantially the following proportions by weight: 20 aluminum seventy parts, zinc twenty-two parts, copper three parts, and antimony five parts.

In producing the alloy, the method which 25 I have found to be the best is as follows. About one-third of the aluminum is melted and raised to a high temperature. The copper is then introduced into the aluminum, and then the balance of the aluminum is introduced into the mass. The temperature of 30 the mass is then lowered and the zinc and then the antimony introduced, the mass being agitated thoroughly to insure the proper mixing of the different metals. The composition will then be ready for casting.

The introduction of the antimony into the mass is for the purpose of overcoming the

shrinkage of the mass when cooling, the increase in volume of the antimony as it cools, counteracting the contraction of the other 40 metals as they cool.

The alloy composed of the above materials combined in the proportions substantially as above set forth, will produce a very satisfactory casting metal, especially well adapted 45 for use in connection with die-casting machines where pressure is used and the resultant articles will be very strong.

What I claim is:

1. A composition of matter comprising 50 aluminum, zinc, copper and antimony.

2. A composition of matter comprising aluminum, zinc, copper and antimony combined in substantially the following proportions by weight: aluminum seventy parts, 55 zinc twenty-two parts, copper three parts and antimony five parts.

3. The method of producing a composition of matter composed of aluminum, zinc, copper and antimony, consisting in melting 60 a portion of the aluminum and raising it to a high temperature, then introducing the copper, then the balance of the aluminum, then lowering the temperature of the mass and introducing the zinc and antimony and 65 thoroughly agitating the mass.

In testimony, that I claim the foregoing as my invention, I have signed my name in presence of two witnesses, this first day of October, 1913.

WILLIAM A. MCADAMS.

Witnesses:

F. GEORGE BARRY,

HENRY C. THIEME.